

# UNITED STATES PATENT OFFICE.

ODUS C. HORNEY, OF THE UNITED STATES ARMY, PHILADELPHIA, PENNSYLVANIA.

## PRIMER FOR CARTRIDGES.

No Drawing.

Application filed July 17, 1925. Serial No. 44,346.

(GRANTED UNDER THE ACT OF MARCH 3, 1883; 22 STAT. L. 625.)

The invention described herein may be used by the Government, or any of its officers or employees in prosecution of work for the Government, or by any other person in the United States, without payment to me of any royalty thereon, in accordance with the act of March 3, 1883.

This invention relates to a primer for cartridges, and has particular reference to the metallic composition thereof.

Primers for the ignition of cartridges and for other purposes must be made of a metal which possesses the characteristic of elasticity so as to readily yield to the blow of the firing pin and of strength to withstand the excessive pressure produced. The material must also possess a high degree of resistance to the chemical action of the ingredients of the igniting charge of the primer.

I have discovered that the foregoing requirements are admirably fulfilled when the

primer is composed of an alloy containing a high percentage of nickel. One example of such an alloy is a material commercially known as "Monel metal" and consists of 25 nickel 75%, copper 23.5% and iron 1.5%.

While the composition cited has been found to have given excellent results it is by no means intended to limit my invention to the ingredients and proportions mentioned in the formula for "Monel metal" but to include suitable alloys containing a high percentage of nickel.

I claim:

1. A primer made of an alloy containing 35 nickel 75%, copper 23.5%, and iron 1.5%.
2. A primer made of a corrosion resisting alloy containing a high percentage of nickel.
3. A primer made of an alloy containing a high percentage of nickel.

ODUS C. HORNEY.